# EUROPEAN PATENT SPECIFICATION

(11) **EP 2 152 919 B1**
(45) Date of publication and mention of the grant of the patent: **30.09.2015**
(21) Application number: 08758587.3
(22) Date of filing: 16.05.2008
(51) Int. Cl.: C21D 9/08, C22C 38/26, C22C 38/28, C22C 38/32, C22C 38/14, C21D 1/25, C21D 9/14, C21D 6/00

(54) **USE OF A STEEL ALLOY FOR WELL PIPES FOR PERFORATION OF BOREHOLE CASINGS, AND WELL PIPE**
VERWENDUNG EINER STAHLLEGIERUNG FÜR BOHRROHRE ZUR PERFORATION VON BOHRLOCHGEHÄUSEN UND BOHRROHR
UTILISATION D'UN ALLIAGE D'ACIER POUR DES TUYAUX DE PUITS POUR LA PERFORATION DE CUVELAGES DE PUITS DE FORAGE, ET TUYAU DE PUITS

(30) Priority: 16.05.2007 DE 102007023306
(43) Date of publication of application: 17.02.2010
(73) Proprietor: Benteler Deutschland GmbH, 33104 Paderborn (DE)
(72) Inventor: PETERS, Andreas, 40625 Düsseldorf (DE); TRITTEL, Rolf, 45897 Gelsenkirchen (DE); HALFPAP, Christopher, 49356 Diepholz (DE)
(74) Representative: Ksoll, Peter
(86) International application number: PCT/EP2008/003961
(87) International publication number: WO 2008/138642

(56) References cited:
- EP-A- 0 753 595
- EP-A- 1 516 934
- EP-A- 1 764 423
- JP-A- 55 134 156
- JP-A- 2001 192 773
- US-A- 4 790 885
- US-A- 5 454 883
- US-A1- 2003 155 052
- US-A1- 2004 035 576
- US-A1- 2004 228 679
- US-A1- 2005 087 269
- US-B1- 6 228 183
- KATSUMATA M ET AL: "DEVELOPMENT OF HIGH STRENGTH AND HIGH TOUGHNESS LOW CARBON - LOW ALLOY STEEL FOR HOT FORGED PARTS" KOBELCO TECHNOLOGY REVIEW, KOBE STEEL, KOBE, JP, no. 11, 1 June 1991 (1991-06-01), pages 29-32, XP001038795 ISSN: 0913-4794

## Description

Perforation units or so-called "perforating guns" are used for opening or renewed opening of boreholes for exploration of liquid or gaseous energy carriers, i.e. for exploration of gas or crude oil, and are made from a well pipe which accommodates an explosive unit. The explosive unit normally includes several hollow charges as well as the necessary ignition electronics. As the explosive charges are ignited in the respective crude-oil-carrying or natural-gas-carrying layer, holes are formed in the well pipe, in the pipe liner arranged in the borehole, and the cement normally filled behind the pipe liner. The natural-gas-guiding or crude-oil-gulding rock formation outside the cement wall of the borehole is perforated by a plasma beam (jet) of the explosive charge so that the crude oil or the natural gas can be introduced via the perforations and holes in the pipe liner into the borehole and discharged upwards.

The well pipes of the perforation units must withstand before use, i.e. during lowering and positioning, In the region of the respective crude-oil-carrying or natural-gas-carrying layer high mechanical stress in the form of high pressure as well as sometimes elevated temperatures that may reach above 266 °C. This requires that the well pipes have a narrow tolerance with respect to their geometric shape, exhibit only a slight eccentricity, and moreover are made of a material of high strength. The yield point should generally range above 600 MPa. Oftentimes, yield points of greater than 890 MPa are required to prevent the collapse of the perforation unit.

During the use of the perforation unit, the high internal pressures which develop, when the explosive charges ignite, demand a high strength, especially a high toughness and in particular a transverse notch impact toughness in order to prevent the well pipe from bursting as a consequence of an uncontrolled crack growth during explosion. The used materials must therefore exhibit a high strength and at the same time also a good toughness.

Exploration of increasingly deeper fossil fuel deposits and the desire to equip perforation units increasingly with stronger explosive charges to create larger and deeper boreholes presupposes that the well pipes are provided of significantly better strength and toughness properties compared to those known from the state of the art and currently available.

The demand for high strength with sufficient toughness at the same time can be basically met using quenched and tempered steels which have a carbon content in the range of 0.25 % to 0.45 %. These steels normally contain further alloying elements, such as, e.g., chromium, molybdenum and nickel which in particular provide optimum capacity for full quenching and tempering.

Quenching and tempering treatment, i.e. hardening and tempering, produces steels with a martensitic structure to realize the wanted combination of strength and toughness as a result of their even and fine microstructure. The strength demanded from the respective component and thus from the material is primarily adjusted by the temperature selection for tempering. Lower tempering temperatures result basically in increased final strength of the material. The rise in strength is accompanied, however, by a decrease in toughness and reduction in ductility. Strength and toughness behave in opposition to one other in metal-physical sense. In other words, the increase in strength set in a material gets higher, for example through selection of a lower tempering temperature is accompanied by a decrease in toughness and ductility. Therefore, there are limits to satisfy the desire for high strength and good toughness properties at the same time.

Many measures were developed and implemented during steel production to produce high-strength steel materials with sufficient toughness at the same time. Enhancements of the metallurgical degree of purity of the materials, production of structures with little segregation and assurance of a fine initial structure before austenitizing are considered among others. The latter is of crucial importance because for metal-physical reasons only fineness of the respective product structure is able to realize a strength increase as well as simultaneously an increase in toughness. All other strength enhancing mechanisms, e.g. solid solution hardening, cold solidification, or precipitation hardening, generally have a toughness-reducing effect.

By optimizing the alloy composition, the steel production process, the hot-rolling conditions, and the final quenching and tempering treatment, a quenched and tempered steel can be produced for example which contains about 0.3 % of carbon, 1.0 % of chromium, and 0.2 % of molybdenum and a remainder of iron and impurities resulting from smelting, and exhibits a tensile strength of 950 MPa and a transverse notch impact toughness of 130 J/cm². The thus described level of strength and toughness reflects the quality potential attainable for this material classification. An improved quality potential cannot be realized for this frequently employed material process with the necessary process reliability, even when further optimizing the afore-mentioned production conditions

The prior art to US 2 586 041 discloses a steel alloy which contains 0.22 to 0.37 of carbon, 0.65 to 0.95 % of manganese, 0.6 to 0.8 % of silicon, 0.7 to 0.9 % of chromium, 0.4 to 0.6 % of molybdenum, 0.7 to 0.95 % of nickel, and 0.003 to 0.006 % of boron, remainder iron and impurities resulting from smelting, and is subjected to a heat treatment which involves a quenching from a temperature above Ac3 and tempering at 204 to 260 °C of the steel for formation of a martensitic structure. In this way, a toughness of more than 20 ft.-lbs (=33.9 J/cm²) at a temperature of -73 °C should be ascertained by a notched bar impact bend test. At the same time, the tensile strength Rm should be greater than 220,000 p.s.i. (= 1,516 MPa). The product of tensile strength and notch impact energy reaches a value of 5,205 ksi*ft. lbs (about 60.822 MPa x J/cm²). Such high-strength steel is intended, for example, for application in landing gears of airplanes, for drill tips of pneumatic drilling tools, and for perforating guns. The steel is characterized primarily by a very high strength. Its toughness at low temperatures is, however, a property which remains ineffective in perforating guns as a result of the significantly higher thermal stress within a borehole. The toughness (28 ft.-lbs = about 47.5 J/cm²) measured at room temperature is relatively small.

The desired tempering temperatures between 204 and 260 °C may further adversely affect the inherent residual stress, in particular when tempering operations have not been entirely completed. Even though this steel alloy has an alloying content of below 4 %, the lower limit is calculated at 3.22 % so that the alloy is very expensive by today's standards, especially because of the high proportion of molybdenum and nickel.

The prior art to JP 55 134156 A discloses steel products for oil well pipe having superior sulfide stress corrosion crack resistance and tensile strength of 60 kg/mm² or more. The composition of steel products is composed of by weight C 0.2 - 0.5 %, Si 0.10 - 0.35 %, Mn 0.5 - 9.90 %, P ≤ 0.015%, S ≤ 0.010 %, Al 0.01 0.10 %, Ca 0.0010 - 0.020 %, and the balance Fe and inevitable-impurities. It May further contain one or more out of Cr 0.1 - 2.0 %, Mo ≤ 0.50 %, Nb 0.05 %, V ≤ 0.10 %, Ti 0.01 - 0.10 %, B 0.0005 - 0.005 %, Cu 0.20 - 0.60 % and Ni 0.10 - 0.60 %.

US 2005/0087288 A1 discloses a method for producing steel line pipe having low yield strength to tensile strength ratio in order to improve the capability of steel line pipe to undergo reeling into coil form and unreeling therefrom. The method includes (a) providing a steel pipe having a composition consisting essentially of in weight percent: C 0.01 to 0.40, Mn 0.25 to 2.0, P residual to less than 0.5, S residual to less than 0.020, Si residual to 2.0, Cu residual to 1.0, Ni residual to 1.0, Cr residual to 2.0, Mo resildual to 1.0, Al 0.010 minimum to less than 1.0, N residual to 0.030, V residual to less than 0.5, B residual to less than 0.02. Ti residual to less than 0.3, an Nb residual to less than 0.3, balance iron and incidental impurities. The pipe is heated to a temperature within the intercritical Ac1 to Ac3 temperature range, cooled to a temperature below the Ms (martensite start) temperature in order to obtain martensite, reheated to a temperature below the Ac1 temperature for a time suifficient to obtain the desired yield strength, tensile strength and yield strength to tensile strength ratio, and then air cooled.

US 2003/0155052 A1 discloses a high strength steel pipe for an air bag and a process for its manufacture. In order to manufacture a steel pipe for an air bag which can cope with Increase in the pressure of gas blown into an air bag and dereases in the well thickness of an accumulator, a steel having a composition, mass %, of: C 0.05 - 0.20 %, Si 0.1 - 1.0 %, Mn 0.20 - 2.0 %, P at most 0.025 %, S at most 0.010 %, Cr 0.05 - 1.0 %, Al at most .10 %, if necessary at least one of Mo: at most 0.50 %, Ni at most 1.5 %, Cu at most 0.5 %, V at most 0,2 %. Ti at most 0.1 %, Nb at most 0.1 °C and B at most 0.005 % and also if necessary, al least one of Ca at most 0.01 %, Mg at most 0.01 % and REM (rare earth elements) at most 0.01 %, and a remainder of Fe and impurities is used to produce a steel pipe, and the pipe is then subjected to cold working to predetermined dimensions, then to heating to a temperature of at least the Ac1 transformation temperature followed by quenching, and then tempering at a temperature no higher than the Ac1 transformation temperature.

JP 2001 192773 A disclosea a possibility to inexpensively produce a line pipe combining excellent strength, toughness and plastic deformability with high efficiency. This steel for a line pipe has a composition containing C of 0.10 to 0.20 %, Si of 1.0 % or less, Mn of 0.3 to 2.5 %, P of 0.015 % or less S of 0.003 % or less, Ti of 0.06 % or less, Al of 0.001 to 0.1 % and N of 0.007 % or less, moreover containing as optional elements, Cr of 1.0 % or less. Mo of 1.0 % of less, Cu of 1.0 % or less, Ni of 1.0 % or less, Nb of 0.05 % or less, V of 0.10 % or less, B of 0.003 % or less and Ca of 0.005 % or less and simultaneously satisfies the following inequality (a) and has a structure containing martensite and bainite in which the average grain size of austenite is 30 to 200 µm or has a tempered structure thereof: Al x (N-Ti/3.4)≤0.0001 (a).

In Katsumata M et al; "Development of high strength and high toughness low carbon - low alloy steel for hot forged parts" Kobelco Technology review, Kobe Steel, ISSN: 0913-4794, no. 11,1 June 1991, p. 29-32 is a disclosure of new steels with high tensile strength (between 0.981 GPa and 1.37 GPa) and high toughness (equivalent to that of quenched and tempered steels in the as-hot forded condition) that were proposed for automobile components. The new steels are low carbon-low alloy steels with carbon contents of 0.06 % to 0.18 % and with a microstructure of martensite and/or bainite. Alloying elements such as manganese, chromium, molybdenum, niobium and boron should be added in order to increase hardenability and consequently to obtain a bainite and/or martensite structure according to the size of forging components and the cooling media, Excellent balance of strength and toughness was obtained in the water-quenched steels.

The invention is based on the object to provide a steel alloy for making well pipes of perforation units for perforation of boreholes as well as well pipes made of such a steel alloy, with the steel alloy having strength and toughness behaviors which, compared to the state of the art, can be better suited to the application at hand, and wherein the property profile is moreover attained with a cost-efficient alloy.

The object is solved by the use of a quenched and tempered steel alloy according to the chemical composition set forth in patent claims 1 and 20.

The respectively dependent patent claims set forth advantageous configurations of the inventive idea that are not self-evident.

It is proposed for producing well pipes of perforation units for perforation of borehole casings to use a steel as defined in claim 1.

Carbon required for formation of martensite is lowered in the used steel alloy to a value between 0.12 % to 0.25% so as to ensure the formation of lath martensite instead of plate martensite, on one hand, and to attain the desired target strength, on the other hand. Target strength is to be understood as relating to the yield point which may lie above 930 MPa, when suitably heat treated. The yield point of the well pipes should lie at least above 895 MPa at tensile strengths of at least 930 MPa. At the same time, a transverse notch impact toughness of above 105 J/cm² at room temperature is adjusted.

The alloying element manganese is added by alloying to assist the solid solution strengthening so that a portion of the carbon content required for attaining high strength values is compensated. Important for the application of the steel is the use of manganese to promote the capacity for full quenching and tempering of the well pipes. The elements titanium and boron also assist in attaining a capacity for full quenching and tempering as well as a further improvement of the toughness of the steel material.

Titanium serves in this context in particular the fixation of nitrogen occurring in steel in order to fully develop the effect of the element boron to enhance hardenability.

A controlled but not necessary admixture of nickel, chromium, molybdenum or vanadium may assist in the formation of a fine structure, so that the toughness of the material can further be increased.

To realize a fine starting structure before martensitic transformation, it has been shown especially advantageous when the total of titanium, niobium and vanadium has a minimum value of 0.03 and 0.08 %. This ensures that the grain growth during austenitizing is limited as a consequence of sufficient formation of fine precipitation, and the tendency for embrittlement, known in the literature, is prevented when admixing micro-alloying elements in lean stoichiometric environment.

The elements molybdenum, nickel and chromium further promote the capacity for full quenching and tempering of the material.

In order to positively influence in particular the transverse notch impact toughness, it is targeted to limit the maximum sulfur content of the steel to 0.005 % and to alloy the steel with 8 to 25 ppm of calcium. As a result, precipitations of toughness-reducing aluminum oxide from the secondary metallurgy are finely dispersed in steel and do not cause unwanted instable crack propagation in particular when exposed to sudden stress.

The quenching and tempering treatment of the steel alloy first involves austenitizing to a temperature above the material-specific transformation temperature Ac3 over a time period of 0.1 to 10 minutes. Austenitizing preferably takes place over a time period between 0.1 and 5 minutes. The austenitizing temperature preferably lies in a range of 25 °C +/- 5 °C above the transformation temperature Ac3. The exact temperature depends on the heating rate which is very high, when inductive heating is involved. The heating rate lies in a range between 1 and 50 K/s. This is followed by a quenching treatment in a medium which ensures sufficient cooling rate for the material and dimensions of the workpiece and results in the formation of more than 95 % martensite, remainder lower bainite. The quenching medium is preferably water. The quenching rate should range between 60 and 500 K/s. The quenched material is then heated starting from room temperature and tempered over a time period of 1 to 25 minutes, preferably between 5 and 15 minutes, at a temperature range between 280 °C and 700 °C, whereby the selected temperature and temperature profile depend in the required target strength. Finally, the material is cooled in air or quenched in water to room temperature.

The well pipes produced from the mentioned steel alloy and the described quenching and tempering process have outer diameters ranging from 30 to 180 mm at wall thicknesses of 6 to 20 mm.

The transverse notch impact toughness A [J/cm²] is plotted by way of example for a pipe having an outer diameter of 73.4 mm at a wall thickness of 9.2 mm and made from the steel according to the invention in quenched and tempered state, i.e. after austenitizing over 5 minutes at 920 °C, quenching in water, and tempering at different temperatures between 450 and 610 °C, at tempering times of less than 10 minutes, as a function of the respective mechanical parameters, i.e. toughness Rm and yield strength Rp0.2. At the same time, the range of common mechanical-technological properties of a conventional quenched and tempered steel is depicted. This comparison steel has the following chemical composition:

| | |
|---|---|
| Carbon | 0.31 % |
| Manganese | 0.75 % |
| Chromium | 1.00 % |
| Molybdenum | 0.18 % |
| Nickel | 0.14 % |

remainder iron and impurities resulting from smelting.

The steel used according to the invention has following composition:

| | |
|---|---|
| Carbon | 0.16 % |
| Silicon | 0.31 % |
| Nitrogen | 0.0088 % |
| Sulfur | 0.0021 % |
| Manganese | 1.40 % |
| Chromium | 0.19 % |
| Vanadium | 0.005 % |
| Nickel | 0.08 % |
| Molybdenum | 0.03 % |
| Titanium | 0.037 % |
| Niobium | 0.039 % |
| Boron | 0.0017 % |
| Ca | 0.0012 % |

remainder iron and impurities resulting from smelting.

As can be seen in the illustration, the tensile strength and yield strength of the steel according to the invention at a certain transverse notch impact toughness is greater than the tensile strength and yield strength of the comparison steel ascertained by many tests. Just like the steel used in the invention, the comparison steel meets the demand for s yield strength above 895 MPa and a transverse notch impact toughness above 105 J/cm². The characteristic material values of the comparison steel exceed, however, only rarely the yield strengths of above 1,000 MPa at transverse notch impact toughnesses which mostly lie below 150 J/cm².

Conversely, the used steel has the property of being especially solid and at the same time sufficiently tough for the special application at hand because its characteristic material values include transverse notch impact toughnesses of above 160 J/cm² at yield strengths of above 900 MPa. Likewise, the steel used in the invention can be adjusted through suitable heat treatment to a yield strength of above 1,000 MPa. In an extreme case, this exemplary material has reached yield strengths of up to 1.142 MPa at a transverse notch impact toughness of 119 J/cm². In particular the last value pair underscores that the used steel excels in meeting the requirements demanded of well pipes of perforation units for perforation of borehole casings. The heat treatment is hereby modified in particular by changing the tempering temperature. For example, the tensile strength of 860 MPa has been realized at a tempering temperature of 610 °C, while the tensile strength of about 1,200 MPa has been realized at a tempering temperature of 450 °C.

The correlation between toughness and strength can be described for predefined upper and lower limits of these characteristic material values by the mathematical product of these characteristic values. The product of tensile strength and transverse notch impact toughness should range from 141,000 to 165,000 MPa* J/cm² for the steel alloy according to the invention at room temperature in the strength range between 750 MPa and 1,200 MPa. The transverse notch impact toughness Av_quer may also be expressed as function of the yield strength (Rp0.2). The steel alloy used in accordance with the invention has the following correlation: $\begin{matrix}Av_quer \left[J/{cm}^{2}\right] = & - 3.7679 * {10}^{- 1} * {\left[Rp⁢0.2 in MPa\right]}^{2} \\ & + 5.3809 * {10}^{- 1} * {\left[Rp⁢0.2 in MPa\right]}^{2} - 5.9505.\end{matrix}$

The coefficient of determination R² lies above 99 % so that the used steel alloy realizes the targeted material properties at very high process reliability.

The crucial factor for reaching the desired material parameters is a heat treatment that is suited to the material so that the structure can be produced with the desired composition. In particular, the martensite portion of the structure must lie above 95 %, comprised of >85 % lath martensite and <15 % plate martensite. The remainder of the structure is formed of lower bainite.

In order to utilize the high potential of the steel according to the invention for reliably realizing an optimum strength-toughness ratio, it has been shown especially advantageous to interrupt quenching below the martensitic end temperature (Mf), before the material is cooled down to room temperature. As a consequence, thermal stress in the structure is kept as small as possible so that toughness-reducing crack formation is again prevented in the microstructure of the alloy.

A well pipe for perforating guns is made from a seamlessly produced tube round which is subjected to the heat treatment set forth in patent claim 11. The tube round can then be supplied, of course, to a further material removing treatment to adjust the desired end geometry.

## Claims

1. Use of a steel alloy for well pipes of perforating units for perforation of borehole casings, with the steel alloy comprised, in mass-%, of
| | | |
|---|---|---|
| Carbon (C) | 0.15 | -0.22 |
| Manganese (Mn) | 1.3 | -1.8 |
| Silicon (Si) | 0.2 | -0.4 |
| Nitrogen (N) | 0.006 | -0.012 |
| Sulfur (S) | | <0.003 |
| Chromium (Cr) | 0.1 | -0.3 |
| Molybdenum (Mo) | | <0.1 |
| Nickel (Ni) | | <0.1 |
| Vanadium (V) | | <0.05 |
| Niobium (Nb) | 0.01 | -0.05 |
| Titanium (Ti) | 0.02 | -0.04 |
| Boron (B) | 0.0015 | -0.003 |
| Calcium (Ca) | 0.0008 | -0.0020 |
and iron as well as impurities resulting from smelting as remainder, wherein the steel alloy is heated at a heating rate of 1-100 K/s to an austenitizing temperature between 10 to 50 °C above its transformation temperature Ac3, and held at this austenitizing temperature between 0.1 and 10 minutes and austenitized, subsequently quenched at a quenching rate of >50K/s, so as to adjust a martensite content of >95 %, wherein the structure is comprised of >85 % lath martensite, <15 % plate martensite, remainder bainite, and wherein the remainder is formed of lower bainite, wherein the structure is then tempered starting from room temperature between 1 and 25 minutes at temperatures between 280 °C and 700 °C, and finally cooled in air or quenched in water to room temperature, wherein the steel has a tensile strength Rm ranging from 850 MPa to 1,200 MPa at transverse notch impact toughnesses in a range between 190 and 105 J/cm² at room temperature, wherein the product of tensile strength and transverse notch impact toughness lies in the strength range between 850 MPA and 1,200 MPa in a range of 141,000 to 165,000 MPa*J/cm².

2. Use according to claim 1, **characterized in that** the alloy satisfies the totals formulas Ti + Nb + V > 0.03 and Ti + Nb + V < 0.08.

3. Use according to claim 1 or 2, **characterized in that** the titanium/nitrogen ratio T/N ranges between 3.4 and 5.

4. Use according to one of the claims 1 to 3, **characterized in that** the heating rate ranges from 1 to 50 K/s.

5. Use according to one of the claims 1 to 4, **characterized in that** the heating is inductive.

6. Use according to one of the claims 1 to 5, **characterized in that** the austenitizing temperature ranges from 25 °C +/- 5 °C above the transformation temperature Ac3.

7. Use according to one of the claims 1 to 6, **characterized in that** the steel alloy is austenitized over a time period between 0.1 and 5 minutes.

8. Use according to one of the claims 1 to 7, **characterized in that** the quenching rate ranges from 60 to 500 K/s after austenitizing.

9. Use of a steel alloy according to one of the claims 1 to 8, **characterized in that** the quenching operation is interrupted when the martensite finish temperature (Mf) falls below by at most 50 °C.

10. Use according to one of the claims 1 to 9, **characterized in that** the steel alloy is tempered between 1 and 12 minutes.

11. Well pipe of a perforation unit for perforation of borehole casings, producible by:
a) preparing a seamless tubular body of a steel alloy comprised, in mass-, of
| | | |
|---|---|---|
| Carbon (C) | 0.15 | -0.22 |
| Manganese (Mn) | 1.3 | -1.8 |
| Silicon (Si) | 0.2 | -0.4 |
| Nitrogen (N) | 0.006 | -0.012 |
| Sulfur (S) | | <0.003 |
| Chromium (Cr) | 0.1 | -0.3 |
| Molybdenum (Mo) | | <0.1 |
| Nickel (Ni) | | <0.1 |
| Vanadium (V) | | <0.05 |
| Niobium (Nb) | 0.01 | -0.05 |
| Titanium (Ti) | 0.02 | -0.04 |
| Boron (B) | 0.0015 | -0.003 |
| Calcium (Ca) | 0.0008 | -0.0020 |
and iron as well as impurities resulting from smelting as remainder,
b) heating the tubular body at a heating temperature of 1-100 K/s to an austenitizing temperature between 10 to 50 °C above its transformation temperature Ac3,
c) holding at this austenitizing temperature between 0.1 and 10 minutes for austenitizing,
d) subsequently quenching at a quenching rate of >50K/s, so as to adjust a martensite content of >95 %, wherein the structure is comprised of >85 % lath martensite, <15 % plate martensite, remainder bainite, and wherein the remainder of the structure is formed of lower bainite,
e) tempering the tubular body starting from room temperature over a time period of 1 and 25 minutes at temperatures ranging from 280 °C and 700 °C,
f) cooling the tubular body in air or quenching in water to room temperature, so that
the tubular body has a tensile strength Rm ranging from 850 MPa to 1,200 MPa at transverse notch impact toughnesses in a range between 190 and 105 J/cm² at room temperature, and wherein the product of tensile strength and transverse notch impact toughness lies in the strength range between 850 MPa and 1,200 MPa in a range of 141,000 to 165,000 MPa*J/cm².

12. Well Pipe according to claim 11, producible in that the following totals formulas are satisfied: Ti + Nb + V > 0.03 and Ti + Nb + V < 0.08.

13. Well Pipe according to claim 11 or 12, producible in that the titanium/nitrogen ratio T/N ranges between 3.4 and 5.

14. Well pipe according to one of the claims 11 to 13, producible in that the heating rate is selected in a range from 1 to 50 K/s.

15. Well pipe according to one of the claims 11 to 14, producible in that the heating is inductive.

16. Well pipe according to one of the claims 11 to 15, producible in that the austenitizing temperature is selected in a range from 25 °C +/- 5 °C above the transformation temperature Ac3.

17. Well pipe according to one of the claims 11 to 16, producible in that the steel alloy is austenitized over a time period between 0.1 and 5 minutes.

18. Well pipe according to one of the claims 11 to 17, producible in that the quenching rate is selected in a range from 60 to 500 K/s after austenitizing.

19. Well pipe of a steel alloy according to one of the claims 11 to 18, producible in that the quenching operation is interrupted, when the martensite finish temperature (Mf) falls below by not more than 50 °C.

20. Well pipe according to one of the claims 11 to 19, producible in that the steel alloy is tempered between 1 and 12 minutes.

## Patentansprüche

1. Verwendung einer Stahllegierung für Mantelrohre von Perforationseinheiten zur Perforation von Bohrlochverrohrungen, wobei die Stahllegierung in Massenanteilen besteht aus:
| | | |
|---|---|---|
| Kohlenstoff (C) | 0,15 | - 0,22 |
| Mangan (Mn) | 1,3 | - 1,8 |
| Silizium (Si) | 0,2 | - 0,4 |
| Stickstoff (N) | 0,006 | - 0,012 |
| Schwefel (S) | | < 0,003 |
| Chrom (Cr) | 0,1 | - 0,3 |
| Molybdän (Mo) | | < 0,1 |
| Nickel (Ni) | | < 0,1 |
| Vanadium (V) | | < 0,05 |
| Niob (Nb) | 0,01 | - 0,05 |
| Titan (Ti) | 0,02 | - 0,04 |
| Bor (B) | 0,0015 | - 0,003 |
| Kalzium (Ca) | 0,0008 | - 0,0020 |
und Eisen sowie erschmelzungsbedingten Verunreinigungen als Rest, wobei die Stahllegierung mit einer Aufheizgeschwindigkeit von 1 - 100 K/s auf eine Austenitisierungstemperatur zwischen 10 bis 50 °C oberhalb ihrer Umwandlungstemperatur Ac3 erhitzt wird und auf dieser Austenitisierungstemperatur zwischen 0,1 und 10 Minuten gehalten und austenitisiert wird, anschließend mit einer Abschreckgeschwindigkeit von > 50 K/s abgeschreckt wird, so dass sich ein Martensitgehalt von > 95 % einstellt, wobei die Struktur aus > 85 % Lanzett-Martensit, < 15 % Plattenmartensit, Rest Bainit besteht und wobei der Rest aus unterem Bainit gebildet ist, wobei die Struktur dann ausgehend von einer Raumtemperatur zwischen 1 und 25 Minuten bei Temperaturen zwischen 280 °C und 700 °C angelassen wird und schließlich auf Raumtemperatur an Luft oder durch Wasserabschreckung abgekühlt wird, wobei der Stahl eine Zugfestigkeit Rm in einem Bereich von 850 MPa bis 1.200 MPa bei einer transversalen Kerbschlagzähigkeit in einem Bereich zwischen 190 und 105 J/cm² bei Raumtemperatur hat, wobei das Produkt aus Zugfestigkeit und transversaler Kerbschlagzähigkeit in dem Festigkeitsbereich zwischen 850 MPa und 1.200 MPa in einem Bereich von 141.000 bis 165.000 MPa*J/cm² liegt.

2. Verwendung gemäß Anspruch 1, **dadurch gekennzeichnet, dass** die Legierung die Summenformeln Ti + Nb + V > 0,03 und Ti + Nb + V < 0,08 erfüllt.

3. Verwendung gemäß Anspruch 1 oder 2, **dadurch gekennzeichnet, dass** das Titan/Stickstoff-Verhältnis T/N sich in einem Bereich zwischen 3,4 und 5 bewegt.

4. Verwendung gemäß einem der Ansprüche 1 bis 3, **dadurch gekennzeichnet, dass** die Aufheizgeschwindigkeit sich in einem Bereich von 1 bis 50 K/s bewegt.

5. Verwendung gemäß einem der Ansprüche 1 bis 4, **dadurch gekennzeichnet, dass** das Aufheizen induktiv ist.

6. Verwendung gemäß einem der Ansprüche 1 bis 5, **dadurch gekennzeichnet, dass** sich die Austenitisierungstemperatur in einem Bereich von 25 °C +/- 5 °C oberhalb der Umwandlungstemperatur Ac3 bewegt.

7. Verwendung gemäß einem der Ansprüche 1 bis 6, **dadurch gekennzeichnet, dass** die Stahllegierung über eine Zeitdauer zwischen 0,1 und 5 Minuten austenitisiert wird.

8. Verwendung gemäß einem der Ansprüche 1 bis 7, **dadurch gekennzeichnet, dass** sich die Abschreckgeschwindigkeit in einem Bereich von 60 bis 500 K/s bewegt, nach der Austenitisierung.

9. Verwendung eine Stahllegierung gemäß einem der Ansprüche 1 bis 8, **dadurch gekennzeichnet, dass** die Abschreckoperation unterbrochen wird, wenn die Martensit-Finish-Temperatur (Mf) um höchstens 50 °C unterschritten wird.

10. Verwendung gemäß einem der Ansprüche 1 bis 9, **dadurch gekennzeichnet, dass** die Stahllegierung zwischen 1 und 12 Minuten angelassen wird.

11. Mantelrohr einer Perforationseinheit zur Perforation von Bohrlochverrohrungen, herstellbar durch:
a) Bereitstellen eines nahtlosen Rohrkörpers aus einer Stahllegierung, die in Massenanteilen besteht aus:
| | | |
|---|---|---|
| Kohlenstoff (C) | 0,15 | - 0,22 |
| Mangan (Mn) | 1,3 | - 1,8 |
| Silizium (Si) | 0,2 | - 0,4 |
| Stickstoff (N) | 0,006 | - 0,012 |
| Schwefel (S) | | < 0,003 |
| Chrom (Cr) | 0,1 | - 0,3 |
| Molybdän (Mo) | | < 0,1 |
| Nickel (Ni) | | < 0,1 |
| Vanadium (V) | | < 0,05 |
| Niob (Nb) | 0,01 | - 0,05 |
| Titan (Ti) | 0,02 | - 0,04 |
| Bor (B) | 0,0015 | - 0,003 |
| Kalzium (Ca) | 0,0008 | - 0,0020 |
und Eisen sowie erschmelzungsbedingten Verunreinigungen als Rest,
b) Aufheizen des Rohrkörpers mit einer Aufheiztemperatur von 1 - 100 K/s auf eine Austenitisierungstemperatur zwischen 10 bis 50 °C oberhalb seiner Umwandlungstemperatur Ac3,
c) Halten auf dieser Austenitisierungstemperatur zwischen 0,1 und 10 Minuten zur Austenitisierung,
d) anschließend Abschrecken mit einer Abschreckgeschwindigkeit von > 50 K/s, so dass sich ein Martensitgehalt von > 95 % einstellt, wobei die Struktur aus > 85 % Lanzett-Martensit, < 15 % Plattenmartensit, Rest Bainit besteht und wobei der Rest der Struktur aus unterem Bainit gebildet ist,
e) Anlassen des Rohrkörpers ausgehend von einer Raumtemperatur über eine Zeitdauer von 1 und 25 Minuten bei Temperaturen zwischen 280 °C und 700 °C,
f) Abkühlen des Rohrkörpers auf Raumtemperatur an Luft oder durch Wasserabschreckung, so dass der Rohrkörper eine Zugfestigkeit Rm in einem Bereich von 850 MPa bis 1.200 MPa bei einer transversalen Kerbschlagzähigkeit in einem Bereich zwischen 190 und 105 J/cm² bei Raumtemperatur hat, und wobei das Produkt aus Zugfestigkeit und transversaler Kerbschlagzähigkeit in dem Festigkeitsbereich zwischen 850 MPa und 1.200 MPa in einem Bereich von 141.000 bis 165.000 MPa*J/cm² liegt.

12. Mantelrohr gemäß Anspruch 11, herstellbar dadurch, dass die folgenden Summenformeln erfüllt sind: Ti + Nb + V > 0,03 und Ti + Nb + V < 0,08.

13. Mantelrohr gemäß Anspruch 11 oder 12, herstellbar dadurch, dass sich das Titan/Stickstoff-Verhältnis T/N in einem Bereich zwischen 3,4 und 5 bewegt.

14. Mantelrohr gemäß einem der Ansprüche 11 bis 13, herstellbar dadurch, dass die Aufheizgeschwindigkeit ausgewählt wird in einem Bereich von 1 bis 50 K/s.

15. Mantelrohr gemäß einem der Ansprüche 11 bis 14, herstellbar dadurch, dass das Aufheizen induktiv ist.

16. Mantelrohr gemäß einem der Ansprüche 11 bis 15, herstellbar dadurch, dass die Austenitisierungstemperatur ausgewählt wird in einem Bereich von 25 °C +/- 5 °C oberhalb der Umwandlungstemperatur Ac3.

17. Mantelrohr gemäß einem der Ansprüche 11 bis 16, herstellbar dadurch, dass die Stahllegierung über eine Zeitdauer zwischen 0,1 und 5 Minuten austenitisiert wird.

18. Mantelrohr gemäß einem der Ansprüche 11 bis 17, herstellbar dadurch, dass die Abschreckgeschwindigkeit ausgewählt wird in einem Bereich von 60 bis 500 K/s, nach der Austenitisierung.

19. Mantelrohr aus einer Stahllegierung gemäß einem der Ansprüche 11 bis 18, herstellbar dadurch, dass die Abschreckoperation unterbrochen wird, wenn die Martensit-Finish-Temperatur (Mf) um nicht mehr als 50 °C unterschritten wird.

20. Mantelrohr gemäß einem der Ansprüche 11 bis 19, herstellbar dadurch, dass die Stahllegierung zwischen 1 und 12 Minuten angelassen wird.

## Revendications

1. Utilisation d'un alliage d'acier pour canalisations de puits d'unités de perforation pour la perforation de cuvelages de puits de forage, l'alliage d'acier comprenant en % en masse les corps suivants :
| | | |
|---|---|---|
| carbone (c) | 0,15 | -0,22 |
| manganèse (Mn) | 1,3 | -1,8 |
| silicium (Si) | 0,2 | -0,4 |
| azote (N) | 0,006 | -0,012 |
| soufre (S) | | <0,003 |
| chrome (Cr) | 0,1 | -0,3 |
| molybdène (Mo) | | <0,1 |
| nickel (Ni) | | <0,1 |
| vanadium (V) | | <0,05 |
| niobium (Nb) | 0,01 | -0,05 |
| titane (Ti) | 0,02 | -0,04 |
| bore (B) | 0,0015 | -0,003 |
| calcium (Ca) | 0,0008 | -0,0020 |
et du fer ainsi que des impuretés résultant de la fusion comme résidu, dans laquelle l'alliage d'acier est chauffé à une cadence de chauffage de 1 à 100 K/s à une température d'austénisation comprise entre 10 et 50 °C au-dessus de sa température de transformation Ac3 et maintenu à cette température d'austénisation entre 0,1 et 10 minutes et austénisé, puis trempé à une cadence de trempe >50 K/s de manière à régler une teneur en martensite >95 %, dans laquelle la structure est constituée d'une quantité >85 % de martensite en lames, d'une quantité <15 % de martensite en plaques, le restant étant de la bainite, et dans laquelle le résidu est formé de bainite inférieure, dans laquelle la structure est ensuite traitée au revenu en partant de la température ambiante entre 1 et 25 minutes à des températures entre 280 °C et 700 °C et enfin refroidi à l'air ou trempé à l'eau à température ambiante, dans laquelle l'acier a une résistance à la traction Rm allant de 850 MPa à 1200 MPa à des résiliences transversales par impact sur barreaux entaillés dans une plage comprise entre 190 et 105 J/cm² à température ambiante, dans laquelle le produit de la résistance à la traction et de la résilience transversale par impact sur barreaux entaillés se situe dans la plage de résistances entre 850 MPa et 1200 MPa dans une plage de 141 000 à 165 000 MPa*J/cm².

2. Utilisation selon la revendication 1, **caractérisée en ce que** l'alliage satisfait aux formules totales Ti + Nb + V > 0,03 et Ti + Nb + V < 0,08.

3. Utilisation selon la revendication 1 ou la revendication 2, **caractérisée en ce que** le rapport du titane à l'azote T/N se situe entre 3,4 et 5.

4. Utilisation selon l'une quelconque des revendications 1 à 3, **caractérisée en ce que** la cadence de chauffage se situe dans une plage de 1 à 50 K/s.

5. Utilisation selon l'une quelconque des revendications 1 à 4, **caractérisée en ce que** le chauffage est inductif.

6. Utilisation selon l'une quelconque des revendications 1 à 5, **caractérisée en ce que** la température d'austénisation se situe 25 °C +/-5 °C au-dessus de la température de transformation Ac3.

7. Utilisation selon l'une quelconque des revendications 1 à 6, **caractérisée en ce que** l'alliage d'acier est austénisé sur une période de temps comprise entre 0,1 et 5 minutes.

8. Utilisation selon l'une quelconque des revendications 1 à 7, **caractérisée en ce que** la cadence de trempe se situe dans la plage de 60 à 500 K/s après austénisation.

9. Utilisation d'un alliage d'acier selon l'une quelconque des revendications 1 à 8, **caractérisée en ce que** l'opération de trempe est interrompue lorsque la température de finition de martensite (Mf) chute en dessous au maximum de 50 °C.

10. Utilisation selon l'une quelconque des revendications 1 à 9, **caractérisée en ce que** l'alliage d'acier est traité au revenu entre 1 et 12 minutes.

11. Canalisation de puits d'une unité de perforation pour la perforation de cuvelages de puits de forage, que l'on peut produire par les étapes consistant à :
a) préparer un corps tubulaire sans soudure d'un alliage d'acier comprenant en pourcentage en masse les corps suivants :
| | | |
|---|---|---|
| carbone (c) | 0,15 | -0,22 |
| manganèse (Mn) | 1,3 | -1,8 |
| silicium (Si) | 0,2 | -0,4 |
| azote (N) | 0,006 | -0,012 |
| soufre (S) | | <0,003 |
| chrome (Cr) | 0,1 | -0,3 |
| molybdène (Mo) | | <0,1 |
| nickel (Ni) | | <0,1 |
| vanadium (V) | | <0,05 |
| niobium (Nb) | 0,01 | -0,05 |
| titane (Ti) | 0, 02 | -0,04 |
| bore (B) | 0,0015 | -0,003 |
| calcium (Ca) | 0,0008 | -0,0020 |
et du fer ainsi que des impuretés résultant de la fusion comme résidu,
et du fer ainsi que des impuretés résultant de la fusion comme résidu,
b) chauffer le corps tubulaire à une température de chauffage de 1 à 100 K/s à une température d'austénisation comprise entre 10 et 50 °C au-dessus de sa température de transformation Ac3,
c) maintenir à cette température d'austénisation entre 0,1 et 10 minutes pour l'austénisation,
d) tremper ensuite à une cadence de trempe >50 K/s de manière à régler une teneur en martensite >95 %, dans laquelle la structure est constituée d'une quantité >85 % de martensite en lames, d'une quantité <15 % de martensite en plaques, le restant étant de la bainite, et dans laquelle le restant de la structure est formée de bainite inférieure,
e) traiter au revenu le corps tubulaire en partant de la température ambiante sur une période de temps de 1 à 25 minutes à des températures de 280 °C à 700 °C, et
f) refroidir le corps tubulaire à l'air ou le tremper à l'eau à température ambiante, de sorte que :
le corps tubulaire ait une résistance à la traction Rm allant de 850 MPa à 1200 MPa à des résiliences transversales par impact sur barreaux entaillés dans une plage comprise entre 190 et 105 J/cm² à température ambiante, et dans laquelle le produit de la résistance à la traction et de la résilience transversale par impact sur barreaux entaillés se situe dans la plage de résistances entre 850 MPa et 1200 MPa dans une plage de 141 000 à 165 000 MPa*J/cm².

12. Canalisation de puits selon la revendication 11, dans laquelle l'alliage satisfait aux formules totales Ti + Nb + V > 0,03 et Ti + Nb + V < 0,08.

13. Canalisation de puits selon la revendication 11 ou la revendication 22, dans laquelle le rapport du titane à l'azote T/N se situe entre 3,4 et 5.

14. Canalisation de puits selon l'une quelconque des revendications 11 à 13, dans laquelle la cadence de chauffage se situe dans une plage de 1 à 50 K/s.

15. Canalisation de puits selon l'une quelconque des revendications 11 à 14, dans laquelle le chauffage est inductif.

16. Canalisation de puits selon l'une quelconque des revendications 11 à 15, dans laquelle la température d'austénisation se situe 25 °C +/-5 °C au-dessus de la température de transformation Ac3.

17. Canalisation de puits selon l'une quelconque des revendications 11 à 16, dans laquelle l'alliage d'acier est austénisé sur une période de temps comprise entre 0,1 et 5 minutes.

18. Canalisation de puits selon l'une quelconque des revendications 11 à 17, dans laquelle la cadence de trempe se situe dans la plage de 60 à 500 K/s après austénisation.

19. Canalisation de puits d'un alliage d'acier selon l'une quelconque des revendications 11 à 18, dans laquelle l'opération de trempe est interrompue lorsque la température de fini de martensite (Mf) chute en dessous de pas plus de 50 °C.

20. Canalisation de puits selon l'une quelconque des revendications 11 à 19, dans laquelle l'alliage d'acier est traité au revenu entre 1 et 12 minutes.
